

## UNITED STATES PATENT OFFICE.

NORMAN B. PILLING, OF WILKINSBURG, PENNSYLVANIA, ASSIGNOR TO WESTINGHOUSE ELECTRIC & MANUFACTURING COMPANY, A CORPORATION OF PENNSYLVANIA.

## METHOD OF TREATING ALLOYS.

No Drawing. Application filed September 2, 1922. Serial No. 585,856.

My invention relates to ferrous alloys, such as silicon and similar steels, more especially to a method of treating such alloys to make them readily workable mechanically.

It is among the objects of this invention to provide a method of treating ferrous alloys which shall render them readily workable by mechanical operations, such as bending, stamping, drawing, shearing or the like.

It is a further object of this invention to provide a method of treating ferrous alloys which shall be simple, inexpensive and practical for use in the commercial adaptation of such ferrous alloys.

It is generally known that silicon imparts to iron or steel hardness and brittleness that render silicon-iron or steel alloys of more than about 4% silicon difficult to work and of little value except in castings. However, silicon-iron or steel alloys have low hysteresis and eddy-current losses and, therefore, are specially advantageous for utilization in the manufacture of transformer cores and armature and stator structures in electrical machines, in which the steel is utilized in thin-sheet form.

I have found that certain grades of silicon steel, such as are used in electro-magnetic devices, exhibit excessive brittleness when an attempt is made to work them. This is made manifest by the inability of the metal sheets to withstand such operations as cutting, shearing, stamping, drawing or similar operations in which a certain amount of ductility is necessary. Brittleness is most commonly encountered in steels having a silicon content in excess of 4.0%, and such alloys will break and split spontaneously when shearing or stamping operations are attempted, leaving a rough ragged edge and rendering the material unusable. The burr may scratch through the sheet insulation in the assembled transformer.

My invention consists in the discovery of the fact that the brittleness may be avoided by conducting the desired operation of deformation at a slightly elevated temperature. Thus, in a particular case in which the silicon steel had a composition Si-4.69% Mn-0.32%, a 14 mil thick sheet was so brittle that a strip bent with the fingers through an angle of 90° cracked in two; when

heated to 100° C. the same sheet could not only be bent, but the bend flattened with a hammer blow without fracture.

It appears that the brittleness which has been noted in silicon steel is a modification of the brittleness which even iron of the highest purity (electrolytic, vacuum fused) develops at sufficiently low temperatures, approximately -110° C. The action of alloyed silicon is to raise the temperature at which brittleness is appreciable, slowly for the first 2% silicon, thereafter at a more rapid rate, until it reaches atmospheric temperatures at about 4% Si. For higher percentages of silicon, an elevation of the temperature at which deformation is attempted, proportioned to the silicon content, yields temporary ductility.

From the discovery that the brittleness is not a peculiar property of iron-silicon alloys, but that it is a modification of the low-temperature brittleness of iron, I have concluded that ductility may be produced in other ferrous alloys in which the alloying elements are in solid solution, by increasing the temperature at which mechanical deformations are conducted. I have found that an iron-aluminum alloy, containing about 7% aluminum, which was so brittle when cold as to be unworkable could be hammered and otherwise deformed at a temperature of 150° C. without difficulty.

Generally, the temperature of treatment of ferrous alloys to give temporary ductility ranges from about 30° to about 200° C.

It will be evident from the above description of my invention that, by treating silicon and other steels in accordance therewith, a larger amount of silicon may be used in commercial electrical steels, since it is possible to readily work the same in the above-described manner. Another advantage of my method of treating ferrous alloys, such as silicon steel, is that the treated metals are not as destructive on dies and other machine tools, resulting in a considerable increase of life which reduces the expense of manufacture.

Although I have described a specific embodiment of this invention, it will be obvious to those skilled in the art that various modifications may be made in the details of the process herein set forth without depart-

ing from the principles thereof. For instance, the working temperatures at which the physical properties of alloys are altered to obtain greater temporary ductility may 5 vary from a temperature somewhat above atmospheric to a temperature below a visible heat. The amount of silicon or other substance permissible in such alloys may be varied to obtain an alloy having desired 10 characteristics. The alloys may contain other ingredients, such as manganese, phosphorus and carbon, which are present as impurities or are added to modify the characteristics of the alloy.

15 I claim as my invention:

1. The method of working iron-silicon alloys containing about 4 to 8% silicon which comprises heating said alloys to a temperature above 30° and below 200° C. and subjecting them to mechanical alterations while 20 within this temperature range.
2. The method of working iron-silicon alloys containing from 4 to 8% silicon which comprises heating said alloys to temperatures above 30° C. and below a visible 25

heat and then subjecting them to mechanical alterations while within this temperature range, the temperature of working being proportional to the amount of alloying metal in said alloys. 30

3. The method of working iron-silicon alloys containing from 4 to 8% silicon which comprises heating said alloys to temperatures above 30° C. and below a visible heat and subjecting them to mechanical alterations while within this temperature range. 35

4. The method of working iron-silicon alloys containing from 4 to 8% silicon which comprises heating said alloys to temperatures above 30° and below 200° C. and then subjecting them to mechanical alterations while within this temperature range, the temperature of working being proportional to the amount of alloying metal in said alloys. 40

In testimony whereof, I have hereunto subscribed my name this 17th day of August, 1922.

NORMAN B. PILLING.